

Feb. 24, 1959

E. R. TOMPKINS

2,875,024

## SEPARATION OF BARIUM VALUES FROM URANYL NITRATE SOLUTIONS

Filed Aug. 27, 1946



2,875,024

## SEPARATION OF BARIUM VALUES FROM URANYL NITRATE SOLUTIONS

Edward R. Tompkins, Oak Ridge, Tenn., assignor to the United States of America as represented by the United States Atomic Energy Commission

Application August 27, 1946, Serial No. 693,329

4 Claims. (Cl. 23—14.5)

This invention relates to a method of processing material containing radioactive barium values in small amount for the separation of the barium activity from extraneous matter such as substances of the kind present in solutions of neutron irradiated uranium, for example, plutonium values and fission products other than barium values. More particularly, this invention relates to a method of separating tracer quantities of barium activity from solutions containing the same by adsorption and selective elution.

As described herein, the isotope of element 94, having a mass of 239, is referred to as  $94^{239}$  and is also called plutonium, symbol Pu. In addition, the isotope of element 93 having a mass of 239 is referred to as  $93^{239}$  and is called neptunium, symbol Np. Furthermore, the term "values" or its equivalent when employed herein with reference to an element is intended to embrace the element and compounds thereof. For example, the term "plutonium values" is intended to include plutonium as well as compounds thereof.

Naturally occurring uranium contains a major portion of  $_{92}\text{U}^{238}$ , a minor portion of  $_{92}\text{U}^{235}$  and small amounts of other substances such as  $\text{UX}_1$  and  $\text{UX}_2$ . When a mass of such uranium is subjected to neutron irradiation, particularly with neutrons of resonance or thermal energies,  $_{92}\text{U}^{238}$  by capture of a neutron becomes  $_{92}\text{U}^{239}$  which has a half life of about twenty-three minutes and by beta decay becomes  $93^{239}$ . The  $93^{239}$  has a half life of about 2.3 days and by beta decay becomes  $94^{239}$ . Thus neutron irradiated uranium contains both  $93^{239}$  and  $94^{239}$ , but by storing irradiated uranium for a suitable period of time, the  $93^{239}$  is converted almost entirely to  $94^{239}$ .

In addition to the above mentioned reaction, the reaction of neutrons with fissionable nuclei such as the nucleus of  $_{92}\text{U}^{235}$  results in the production of a large number of radioactive fission products. For example, when an atom of  $_{92}\text{U}^{235}$  undergoes fission, two fragments are formed. These fragments vary sufficiently in their masses and hence their atomic numbers to give some 34 elements, all of which initiate further reaction chains with the emission of radiations. These chains are the source of all of the radioactivity that renders isolation of any one of the products of irradiation of uranium so difficult. The radiations include; (1) beta or high speed negative electrons with variable energy contents, and therefore, different velocities, (2) soft gamma, or electro-magnetic radiation similar to X-rays but with a shorter wave length and moderately higher energy content, (3) hard gamma similar to the soft type except that it has a shorter wave length and higher energy content, and (4) neutrons.

In general, the stability of an atom depends on the ratio of protons to neutrons in the nucleus and certain ratios, therefore, result in an excess energy content that must be emitted as radiation before a stable end product is formed. While most naturally occurring isotopes are

stable and therefore not radioactive, those resulting from fission have proton-neutron ratios such as to cause internal instability. As a result, they tend to stabilize and in the process emit their excess energies in one of five general ways.

In the first place, an atom may emit a beta particle from the nucleus where the only possible source of a negative electron is from a neutron which gives both a positive and negative charge. The loss of the negative charge converts the neutron to a proton and there is a gain of one in atomic number and hence a transmutation to the next higher element. Such a change, of course, alters the proton to neutron ratio and may result in a stable atom, although this is not necessarily true.

15 In the second place, a beta particle of lower energy content may be emitted, thus forming the next higher element while still leaving the nucleus with too great an energy content to be stable. The first beta particle may then be followed by another one to form the second higher element in the atomic series which again may or may not be stable.

20 Thirdly, a beta particle of intermediate energy may be emitted to form an unstable isotope of the next higher element which, due to its excess energy, may give off a gamma ray rather than a beta particle. This process may also result in either stable or an unstable atom.

25 Fourthly, the beta-decay of a fission product may leave the nucleus in a state of excitation higher than the binding energy of a neutron in that nucleus. The neutron is then immediately emitted, and the rate of decay of the neutron-emitting activity observed is just that of the preceding beta activity.

30 Finally, an unstable atom may emit a gamma ray which strikes an electron in one of the inner shells of 35 electrons and ejects it in such a condition that it has some of the properties of the nuclear beta particle. Since the electron, which in this case is known as photoelectron, does not originate in the nucleus, there is no change in the atomic number and the process, like that involved 40 in the emission of a gamma ray, is known as internal conversion.

With the exception of elements 43 and 61, the fission products formed by the above discussed reaction are all 45 well known elements with normal chemical properties, the only point of difference between them and the natural element being that they are composed of unstable isotopes. As brought out above, due to their internal instability they either undergo transmutation to other elements or stabilize themselves internally by the emission of one or more of the previously-mentioned radiations. Consequently, stabilization may involve no change in atomic number or a change of several units. The average length of the fission chains, that is the number of transmutations, is about 3.2 but some may be 55 as long as 6. In general, a chain reaction has emitted a total of 25 to 30 m. e. v. as radiation by the time it is complete.

The fission of  $_{92}\text{U}^{235}$  yields two general types of elements, namely heavy and light. The light fission products possess atomic numbers between 30 and 46 and include radioactive zinc, gallium, germanium, arsenic, selenium, bromine, krypton, rubidium, strontium, yttrium, zirconium, columbium, molybdenum, 43, ruthenium, rhodium, and palladium.

60 The heavy fission products resulting from neutron irradiation of  $_{92}\text{U}^{235}$  possess atomic numbers ranging from 47 to 63 and include radioactive silver, cadmium, indium, tin, antimony, tellurium, iodine, xenon, cesium, barium, lanthanum, cerium, praseodymium, neodymium, 61, samarium and europium.

65 Generally speaking, the irradiation of uranium is conducted under such conditions as result in the combined

amount of neptunium and plutonium being equal to approximately 0.02% by weight of the uranium mass. The concentration of the fission products in neutron irradiated uranium is approximately the same as that of the total of the plutonium and neptunium. However, since many of the fission products are radioactive, they change to other elements at certain fixed rates which are characteristic of each fission product. In other words, they have fixed decay rates. Plutonium, on the other hand, is relatively stable, and since the fission products have varying decay rates, the concentration of the initially formed radioactive fission products with respect to plutonium changes substantially during the course of the reaction and particularly during the storage period which is generally employed after the neutron irradiated uranium has been removed from the reaction zone.

The quantities of the various individual radioactive fission products present in neutron irradiated uranium are extremely small and are generally referred to in the art as "tracer quantities."

As used herein, the terms "tracer" and "tracer quantity" or their equivalents are employed as definitive of extremely small amounts of radioactive materials. For example, radioactive materials in concentrations of  $10^{-10}$  to  $10^{-14}$  molar are considered to be tracer quantities. Such extremely small amounts are incapable of identification by ordinary micro analytical methods, and are, therefore, generally identified by the radiations emitted therefrom by means of any of the usual counting mechanisms known to the art.

As illustrative of a typical neutron irradiated mass containing fission products the following tables are given:

TABLE A

*Distribution of beta activity in neutron irradiated uranium for each fission element as percentage of total*

| Element | Cooling Time |         |          |
|---------|--------------|---------|----------|
|         | 30 Days      | 60 Days | 100 Days |
| Ce..... | 15           | 20      | 27       |
| Sr..... | 18           | 24      | 26       |
| Y.....  | 17           | 22      | 23       |
| Zr..... | 6.8          | 9.6     | 12       |
| Ru..... | 2.6          | 3.4     | 3.5      |
| Ob..... | 1.3          | 2.2     | 3.4      |
| Pr..... | 8.0          | 3.9     | 0.72     |
| Cs..... | 0.15         | 0.33    | 0.72     |
| La..... | 13           | 5.5     | 0.72     |
| Te..... | 0.87         | 0.86    | 0.67     |
| Ba..... | 9.5          | 4.0     | 0.52     |

TABLE B

*Distribution of effective gamma activity in neutron irradiated uranium for each fission element as percentage of total*

| Element | Cooling Time |         |          |
|---------|--------------|---------|----------|
|         | 30 Days      | 60 Days | 100 Days |
| Ob..... | 14           | 30      | 40       |
| Zr..... | 18           | 25      | 26       |
| Ce..... | 4.4          | 6.6     | 10       |
| Ru..... | 7.5          | 9.0     | 8.6      |
| Sr..... | 6.3          | 6.9     | 4.8      |
| La..... | 38           | 16      | 2.3      |
| Y.....  | 1.8          | 2.4     | 2.3      |
| Te..... | .85          | 0.70    | 0.79     |
| Cs..... | .15          | 0.30    | 0.55     |
| Ba..... | 4.1          | 1.8     | 0.24     |
| Pr..... | 1.9          | 0.4     | -----    |
| I.....  | 1.1          | 0.15    | -----    |

As illustrative of the method of obtaining the data for the above tables, the following is given. A mixed fission product solution is subjected to counting and is found to have a total beta activity of 453,600 counts/minute/milliliter. To a 1.00 ml. sample is added 20.0 mg. of Ru and by appropriate chemical manipulation the Ru is isolated and purified. The final precipitate of metallic

Ru weighs 18.0 mg. and gives 4950 counts/minute. The chemical yield is therefore 90% and the count, corrected for chemical yield, is 5500 counts/minute or 1.21% of the total activity.

From the above tables it can be seen that certain fission products are listed as both beta emitters and gamma emitters. This situation results from the presence in neutron irradiated uranium of various isotopes of the elements which comprise the fission products. Thus, one isotope of an element may be a beta emitter while another isotope may be a gamma emitter. Furthermore, and as is more generally the case, certain of the isotopes may emit both types of radiation.

Some members of both the light and heavy groups of fission products may be readily separated from the neutron irradiated uranium mass in that they have been found to have chemical properties similar to the rare earths and can, therefore, be isolated by precipitation under carefully controlled conditions with about one hundred times their weight of carriers such as lanthanum fluoride, bismuth phosphate, and the like. However, many of the fission products in both groups do not respond to such treatment and considerable difficulty has been experienced not only in attempting to separate plutonium values from these fission products, but also in attempting to isolate certain of the fission product values in carrier-free radioactive form.

It can be seen from the above discussion that the separation and isolation of the various products formed as a result of the neutron irradiation of uranium is an extremely difficult task, particularly in view of the fact that extremely small quantities of the individual fission products are present in the materials under treatment. The problem is further complicated by the presence of the various isotopes and the fact that the elements, considered to be formed at the time of fission, may actually represent conversion products from certain of the fission products which have undergone extremely rapid change; that is, those fission products having extremely short half lives. In this connection, approximately 155 isotopes of the fission products involved have been identified and about 30% of these have half lives of over eight hours. Fission products have been identified that have half lives ranging from about 3 seconds to  $10^4$  years.

Since, as pointed out above, the fission product values contained in a solution of neutron irradiated uranium even after a considerable period of storage exhibit radioactive properties, it is particularly advantageous not only to separate these fission product values from plutonium values, but it is also advantageous in certain instances to isolate certain of the fission product values in carrier-free radioactive form in that they serve as an excellent source of radioactivity which may be utilized, among other things, in various fields such as medicine and metallurgy.

Among the fission product values which it is desirable to isolate is radioactive barium. It has been found that barium is present in the above described group of radioactive fission products in comparatively low proportion by weight. Since the percentage of fission products in the overall mass is extremely small, it can be readily seen that the quantity of barium present in the overall mass to be treated is such as to be considered a tracer quantity.

It is an object of this invention to provide a new method for the separation and recovery of barium values.

Another object of this invention is to provide a process for separating radioactive barium values from an irradiated mass containing plutonium values as well as fission product values other than those of barium.

Still another object of this invention is the provision of a method of separating barium values from a solution containing the same by adsorption and selective elution.

It is a further object of this invention to provide an all adsorption process of separating barium values from

a solution containing the same which process may be conveniently operated under conditions of remote control.

These and other objects will become apparent to the skilled worker in the art upon becoming familiar with the following description.

I have found that barium values may be recovered in high concentration from solutions containing the same together with material including fission product values other than barium by a method which comprises passing the solution through an adsorbent under conditions favoring adsorption of barium values together with other material, selectively eluting barium values and certain of the other material present from the adsorbent, passing the resulting eluate through a smaller body of adsorbent under conditions favoring adsorption of barium values and selectively eluting barium values from the smaller body of adsorbent.

In the practice of my invention a wide variety of adsorbents may be utilized including both inorganic adsorbents—such as silica gel, diatomaceous earth, or the like—and organic adsorbents—such as activated carbon, sulphonated carbonaceous material (zeo-carb), phenol-formaldehyde resins preferably containing free sulphonate acid groups, and the like. Particularly advantageous results are obtained in the first portion of the process by the use of ion exchange adsorbents, in which the cation of the adsorbent is exchanged for a similarly charged ion of the substance to be adsorbed. It has been found that the process is particularly effective where the adsorbent used is a relatively inert organic material containing free sulphonate acid groups. Thus, the adsorbent may comprise phenol-formaldehyde resins, lignite, phenol-tannic acid resins, or the like, which contain numerous  $R-SO_3-R'$  groups, in which  $R$  is an organic group such as a methylene group and in which  $R'$  is hydrogen or a metal ion, although  $R'$  is preferably  $H^+$  or  $Na^+$ . A particularly satisfactory adsorbent which may be employed is a phenol-formaldehyde condensation product containing methylene sulphonate acid groups ( $-CH_2SO_3H$ ). In the adsorption process, the hydrogen of the sulphonate acid group is replaced by a cation of the substance to be adsorbed which thereupon forms a more or less loosely associated molecule with the residue.

As an example of a method by which a sulphonated resin may be prepared, 175 parts of 1-hydroxybenzene-4-sulphonate acid are heated together with 40 parts of a formaldehyde solution of 30% strength for one-half hour to about 105° C. Then, further 60 parts of formaldehyde are added and the temperature is kept for about ten hours at 90° C. A hard black resin is formed which is stable to water and of conchoidal fracture. This resin is washed with water and ground to a powder. By regeneration with an acid or a solution of common salt, this base-exchanging body regains its original adsorption capacity.

My invention may be more readily understood by reference to the accompanying drawing in which the figure is a diagrammatic view of an apparatus which may be utilized in the practice of my invention.

Referring to the drawing, the system comprises feed line 1, controlled by valve 2, which passes into tank 3 to the upper portion of which are connected line 4, controlled by valve 5, and line 6, controlled by valve 7. Passage from the bottom of tank 3 is provided by line 8, controlled by valve 9, which line connects to the upper portion of column 10 containing a suitable adsorbent 11. To the upper portion of column 10 are also connected line 12, controlled by valve 13, and line 14, controlled by valve 15. Line 16 connects the lower portion of column 10 to line 17, controlled by valve 18, and to line 19, controlled by valve 20, line 19 passing into header 21 which has connected to the upper portion thereof line 22, controlled by valve 23, and line 24, controlled by valve 25. The bottom of header 21 is connected to the upper portion of column 28 by means

of line 26, controlled by valve 27. Column 28 contains a suitable adsorbent 29 which may be the same as the adsorbent utilized in column 10 or if desired, may be of a different type. To the top of column 28 are connected line 30, controlled by valve 31, and line 32, controlled by valve 33. The bottom of column 28 has connected thereto line 34 which connects to line 35, controlled by valve 36, and to line 37, controlled by valve 38.

In view of the extreme radioactivity of the material under treatment in accordance with my invention, the apparatus diagrammatically illustrated is generally enclosed in a suitable shielding and each of the valves designated above is operated by means of remote control.

In operation of the system described above, the solution containing barium activity is admitted into the system through line 1 by opening valve 2. The solution in tank 3 is then adjusted to a condition favoring the adsorption of barium activity therefrom. For instance, should the concentration of the solution require adjustment or should the pH of the solution require adjustment, the necessary reagents may be introduced into tank 3 through line 6 by opening valve 7. If desired, a plurality of reagent lines may be included in the system for separately introducing various reagents. Agitation of material in tank 3 may be provided by means of air introduced through line 4, controlled by valve 5, and when the solution has reached the desired condition, the air may be utilized to force the solution out of tank 3 through line 8, controlled by valve 9.

When the solution has reached the desired condition, valve 9 is opened, and the solution passes through line 8 into column 10 where barium values together with other material such as fission product values are adsorbed upon the adsorbent bed 11. When the solution under treatment is a uranyl nitrate solution, some  $UO_2^{++}$  ion may be adsorbed in column 10. The unadsorbed material passes through line 16 and 17 to disposal, valve 18 being open and valve 20 in line 19 being closed. After allowing sufficient time for the desired adsorption to take place, elution of  $UO_2^{++}$  is accomplished by passing dilute  $H_2SO_4$  through line 12 controlled by valve 13, and with valve 20 in line 19 closed and valve 18 in line 17 open the eluate from column 10 is passed through lines 16 and 17 to disposal.

Following the elution of  $UO_2^{++}$  as indicated above, valve 15 in line 14 is opened to admit into column 10 citric acid at a concentration and pH sufficient to elute from adsorbent 11 barium values together with other fission product values. While the elution of barium values is being effected valve 18 is closed and valve 20 in line 19 is opened allowing the eluate from column 10 to pass into header 21. In header 21, the pH of the eluate from column 10 is adjusted by the admission of reagent through line 22 controlled by valve 23. The solution is also diluted by the admission of diluent such as water through line 24 controlled by valve 25. Upon reaching the desired pH and desired dilution, valve 27 is opened to allow the thus conditioned solution to pass through line 26 into column 28 wherein adsorption of barium values upon adsorbent 29 takes place. In addition to barium values, certain rare earth values are adsorbed in column 28. Citric acid at a pH of approximately 3 is admitted into column 28 through line 30 by opening valve 31. The citric acid at this concentration selectively elutes the rare earth values thus separating the bulk of the unwanted gamma emitters from the barium values. The eluate from this elution is withdrawn from the column through line 34 and line 35, valve 36 being open and valve 38 in line 37 being closed.

After eluting the undesired material in this manner, valve 36 is closed, valve 38 is opened and citric acid at a pH of approximately 6 is introduced into the column through line 32 by opening valve 33. Citric acid at this pH selectively elutes barium from the adsorbent and the barium values is withdrawn from the column through

lines 34 and 37. The process of my invention may be considered to be comprised of three operations which are extraction of the barium values from uranyl nitrate, concentration and then decontamination. For all practical purposes, the concentration and decontamination are carried out nearly simultaneously. Generally speaking, the dilution which is effected in header 21 is advantageously carried out under such conditions that the final volume of liquid is at least 8 times the volume of the original eluate from column 10.

In selectively eluting the unwanted fission product values from column 28, citric acid at a pH of between 2.3 and 3.5 is advantageously employed. Particularly advantageous results have been obtained at pH's of approximately 3. Whereas citric acid at a pH of 5 to 7 may be advantageously employed as an eluting agent selective for barium. Particularly advantageous results may be obtained in eluting barium with citric acid at a pH of 6.

Generally speaking, the rate of flow of the various liquids through the system is maintained low such as from 1 to 10 ml. per minute per square cm. of adsorbent. Ordinarily the rate of flow of the initial solution through the original column is maintained between 1 to 2 ml. per minute per square cm. of adsorbent. Generally speaking, the rate of flow of eluting agents is a bit higher than that of the initial solution. Advantageous results have been obtained by passing the eluting agents through the column at a rate of flow of between 2 ml. per minute per square cm. to 5 ml. per minute per square cm.

In the practice of my invention, when separating barium values from uranyl nitrate solutions it is advantageous to maintain the concentration of free  $\text{HNO}_3$  in the solution at less than 0.2 M. Although separation of barium values may be effected from solutions in which the free  $\text{HNO}_3$  concentration is greater than 0.2 M, increase in such concentration may cause chemical action on the adsorbent.

While the concentration of the uranyl nitrate solutions which may be processed in accordance with my invention may vary, advantageous results may be obtained by processing a solution having a concentration of between 5% and 30%. Particularly advantageous results have been obtained in processing solutions containing 10 to 20% by weight of uranyl nitrate.

While the temperature at which the process is carried out is also subject to variation, generally speaking, particularly advantageous results may be obtained by operating at normal room temperature. My invention may be more readily understood by reference to the following specific examples.

#### EXAMPLE I

5 liters of a 10% uranyl nitrate solution was passed through an adsorption column containing 1 liter of an ion exchange resin characterized by having a plurality of  $-\text{CH}_2\text{SO}_3\text{H}$  groups and having a particle size of 40-60 mesh. The rate of flow of the solution through the adsorbent was maintained at 1.4 ml. per minute per square cm.

Thereafter 4.0 liters of 0.25 M  $\text{H}_2\text{SO}_4$  was passed through the adsorbent at a rate of flow of 3.2 ml. per minute per square cm. Thereafter 0.5 liter of  $\text{H}_2\text{O}$  was passed through the adsorbent at a rate of flow of 3.2 ml. per minute per square cm. The combined eluate was analyzed and found to contain 5% uranium sulfate and 1% barium. 3.5 liters of 5% citric acid at a pH of 6 was passed through the adsorbent at a rate of flow of 3.2 ml. per minute per square cm. The first 1.7 liters of the resulting eluate were discarded and the remaining 1.8 liters were collected together with the eluate resulting from the passage of 1 liter of water through the column at a rate of flow of 3.2 ml. per minute per square cm. The eluate from the citric acid wash was diluted to an 0.5% citric acid with  $\text{H}_2\text{O}$  and adjusted to a pH of 2.5 with HCl, and passed through a 100 ml. column

containing the same ion exchange resin as was contained in the liter column. The rate of flow through this column was maintained at 8 ml. per minute per square cm. Following adsorption of barium values and other fission product values from 0.5% citric acid solution, 800 ml. of 5% citric acid at a pH of 3.1 were passed through the 100 ml. column at a rate of flow of 1 ml. per minute per square cm. The eluate was collected, and following this elution, 100 ml. of 5% citric acid at a pH of 6 was passed through the column and the eluate discarded. Thereafter 150 ml. of 5% citric acid at a pH of 6 was passed through the column at a rate of flow of 1 ml. per minute per square cm. and this eluate was collected and combined with the eluate resulting from the subsequent passage of 50 ml. of water at a rate of flow of 2 ml. per minute per sq. cm. This eluate contained about 90% of the  $\text{Ba}^{140}$  originally present.

#### EXAMPLE II

125 liters of a 20% uranyl nitrate solution was passed through a 77 liter adsorbent bed of a 40-60 mesh ion exchange resin characterized by having a plurality of  $-\text{CH}_2\text{SO}_3\text{H}$  groups at a flow rate of 1.5 ml. per minute per square cm. Thereafter the adsorbent was washed with 308 liters of 0.25 M  $\text{H}_2\text{SO}_4$  at a flow rate of 3 ml. per minute per square cm. and 77 liters of  $\text{H}_2\text{O}$  at a flow rate of 3 ml. per minute per square cm. The resulting eluate upon analysis contained approximately 5% uranium sulfate and was discarded to waste. Following this elution, the resin bed was washed with 131 liters of 5% citric acid at a pH of 6, the flow rate being maintained at 3 ml. per minute per square cm. The resulting eluate was discarded and thereafter 139 liters of 5% citric acid at a pH of 6 was passed through the adsorbent bed at a flow rate of 3 ml. per minute per square cm. The resulting eluate was collected and combined with the eluate resulting from washing the adsorbent with 77 liters of  $\text{H}_2\text{O}$  at a flow rate of 3 ml. per minute per square cm. This citric acid eluate was diluted to 0.5% citric acid with  $\text{H}_2\text{O}$  and adjusted to a pH of 2.5 with 9 liters of concentrated HCl. The resulting solution of approximately 1400 liters of 1/2% citric acid concentration at a pH of 2.5 was passed through a 7.7 liter volume of the same adsorbent as utilized in the first adsorbent bed at a flow rate of 9 ml. per minute per square cm. The effluent from the adsorbent was discarded. Thereafter the adsorbent was washed with 5% citric acid at a pH of 3.1. 61.6 liters of this solution were passed through the adsorbent at a flow rate of 1 ml. per minute per square cm. Thereafter 8 liters of 5% citric acid at a pH of 6 was passed through the adsorbent bed at a flow rate of 1 ml. per minute per square cm. and the eluate was combined with the 5% citric acid eluate to obtain a rare earth fraction.

16 liters of 5% citric acid at a pH of 6 were passed through the adsorbent bed at the flow rate of 1 ml. per minute per square cm. The adsorbent bed was then washed with 8 liters of water at a flow rate of 3 ml. per minute per square cm. The eluates were combined to obtain a fraction containing the bulk of the  $\text{Ba}^{140}$  originally present.

In the practice of my invention, if desired, increased concentration of barium values may be obtained by utilizing a plurality of successively smaller columns in the concentration and decontamination step. In other words, after extraction on the first column, the resulting barium containing eluate from the first column may be passed a number of times through successively smaller columns using a resin bed volume  $1/10$  of that used in the preceding cycle until the desired reduction of volume is attained.

The process of my invention results in the neater, faster, less dangerous method of separating barium values in that the system for accomplishing the separation is more adapted to handling by remote control and is readily assembled.

In the specification and claims the following terms have the following meanings.

The term "effluent" or its equivalent is intended to include any material coming off of the columns.

The term "eluate" or its equivalent is intended to include any effluent bearing a desired product from a column.

The term "eluting agent" or its equivalent is intended to include a material which removes adsorbed values from a column.

The term "eluting agent" or its equivalent is intended to remove components from the solution. It is to be understood, however, that the invention is not to be limited in any sense by the theory upon which the process is based and that this term is used as it is generally employed in the art of chromatographic separation.

While the invention has been described with reference to certain particular embodiments and with reference to certain specific examples, it is to be understood that the invention is not to be limited thereby. Therefore, changes, omissions, and/or additions may be made without departing from the spirit of the invention as defined in the appended claims which are intended to be limited only as required by the prior art.

I claim:

1. A method of separating barium values from a solution containing the same which comprises passing said solution through an adsorbent under conditions favoring adsorption of barium values together with other material present in said solution, washing said adsorbent with dilute sulfuric acid to remove at least a portion of said other material, washing said adsorbent with citric acid at a pH of approximately 5 to 7 to remove barium values and at least a portion of remaining other material, adjusting the resulting eluate to a pH of approximately 2.3 to 3.5 and diluting said eluate, passing said diluted eluate through a second adsorbent of smaller volume, and selectively eluting said barium values from said second adsorbent.

2. A method of separating barium values from a solution containing uranium values, barium values, and values of fission products other than barium, which comprises passing said solution through an ion exchange resin to adsorb thereon barium values, uranium values and fission product values other than barium values, eluting uranium values from said resin with dilute sulfuric acid, eluting

barium values and at least a portion of said fission product values other than barium values with citric acid at a pH of 6, adjusting the pH of the resulting eluate to about 2.5 with HCl and diluting said eluate at least 8 fold with water, passing said diluted eluate through a smaller volume of said ion exchange resin to adsorb barium values and at least a portion of the remaining fission product values, eluting said adsorbed remaining fission product values with citric acid at a pH of 3, and eluting barium values from said resin with citric acid at a pH of 6.

3. A method of separating  $Ba^{140}$  from a uranyl nitrate solution which also contains  $UO_2^{++}$  and fission product values including rare earth values which comprises passing said solution through an ion exchange resin to adsorb thereon  $UO_2^{++}$ ,  $Ba^{140}$  and fission product values, passing dilute sulfuric acid through said resin to elute therefrom  $UO_2^{++}$ , passing citric acid at a pH of 6 through said resin to elute  $Ba^{140}$  and at least a portion of said fission product values including rare earth values, adjusting the pH of the resulting eluate to 2.5 and diluting said eluate at least 8 fold, passing said diluted eluate through a smaller volume of said resin to adsorb thereon  $Ba^{140}$  and rare earth values, eluting said rare earth values with citric acid at a pH of 3, and eluting said  $Ba^{140}$  with citric acid at a pH of 6.

4. A method of separating  $Ba^{140}$  from a uranyl nitrate solution containing the same together with other material resulting from the fission of  $U^{235}$  which comprises adjusting the concentration of said solution to between 10 and 20% in uranyl nitrate, slowly flowing said solution through an ion exchange resin to remove therefrom  $UO_2^{++}$ , barium values and fission product values, washing said resin with dilute sulfuric acid to remove  $UO_2^{++}$ , eluting barium values and at least a portion of said fission product values with citric acid at a pH of 6 and adjusting the pH of said citric acid eluate to about 2.5 with HCl, diluting said adjusted eluate at least 8 fold with water, passing said diluted eluate through about  $\frac{1}{10}$  the volume of said ion exchange resin to adsorb barium values and rare earth values, eluting said rare earth values with citric acid at a pH of 3 and eluting said barium values with citric acid at a pH of 6.

No references cited.

UNITED STATES PATENT OFFICE  
CERTIFICATE OF CORRECTION

Patent No. 2,875,024

February 24, 1959

Edward R. Tompkins

It is hereby certified that error appears in the printed specification of the above numbered patent requiring correction and that the said Letters Patent should read as corrected below.

Column 6, line 51, for "eluae" read -- eluate --; column 9, lines 9 and 10, for "The term "eluting agent" or its equivalent is intended moval" read -- The term "adsorption" is utilized in referring to removal --.

Signed and sealed this 8th day of September 1959.

(SEAL)

Attest:

KARL H. AXLINE  
Attesting Officer

ROBERT C. WATSON  
Commissioner of Patents

UNITED STATES PATENT OFFICE  
CERTIFICATE OF CORRECTION

Patent No. 2,875,024

February 24, 1959

Edward R. Tompkins

It is hereby certified that error appears in the printed specification of the above numbered patent requiring correction and that the said Letters Patent should read as corrected below.

Column 6, line 51, for "eluae" read -- eluate --; column 9, lines 9 and 10, for "The term "eluting agent" or its equivalent is intended removal" read -- The term "adsorption" is utilized in referring to removal --.

Signed and sealed this 8th day of September 1959.

(SEAL)

Attest:

KARL H. AXLINE  
Attesting Officer

ROBERT C. WATSON  
Commissioner of Patents